

## UNITED STATES PATENT OFFICE

RICHARD S. McCLAUGHRY, OF WHITING, INDIANA, ASSIGNOR TO STANDARD OIL COMPANY, OF WHITING, INDIANA, A CORPORATION OF INDIANA

## GRINDING COMPOUND

No Drawing.

Application filed January 12, 1928. Serial No. 246,392.

This invention relates to grinding compounds suitable for use in preparing surfaces of high pressure apparatus, valves of internal combustion engines and similar purposes.

According to the present invention the grinding compound contains an abrasive, a wax, mineral oil and alkali sulfates derived from oils preferably mineral oil. The grinding compounds may, if desired, include small quantities of water and soap and may be reduced in consistency to the desired extent by the addition of a small quantity of mineral oil of low viscosity.

I have further discovered that grinding compounds are greatly improved with respect to the speed of grinding and also with respect to the finish obtained, by using a plurality of abrasives of different degrees of hardness, the softer abrasives being used in the form of relatively coarse particles and the harder abrasives being used in relatively fine state.

It is preferred to use preferentially oil soluble sulfonates derived from mineral oil. These sulfonates may be produced by adding a small quantity of alkali to acid treated petroleum oil after withdrawal of sludge and extracting with dilute alcohol or acetone, in the manner described in Humphreys' Patent No. 1,286,179. Alkali sulfonates derived from other oils, and preferentially water soluble sulfonates derived from mineral oils may be used if desired.

As the wax it is preferred to employ petrolatum, for example, a petrolatum of a melting point about 110° F. or higher. Other solid waxes may be used if desired; for example, paraffin wax.

As the abrasive it is preferred to employ carborundum in finely divided form. Other abrasives may, however, be employed, if desired. Where a hard and a somewhat softer abrasive are employed, it is preferred to employ carborundum and emery. The size of the abrasive particles may vary considerably

in accordance with the work for which the material is to be employed. As a general rule the carborundum may suitably be between 150 and 220 mesh while the emery may be somewhat larger, for example, between 80 and 100 mesh.

The invention will be more completely understood from the following examples:

## Example I

|                                                                                                                 | Per cent |
|-----------------------------------------------------------------------------------------------------------------|----------|
| Alkali compounds of preferentially oil soluble sulfonic acids derived from mineral oil (50% sulfonates 50% oil) | 30       |
| Petrolatum (melting point 116° F.)                                                                              | 30       |
| Carborundum (150-220 mesh)                                                                                      | 30       |
| Fatty acid soap                                                                                                 | 3        |
| Water                                                                                                           | 0.5      |
| Straw oil                                                                                                       | 3.5      |

## Example II

|                                                                                                                 | Per cent |
|-----------------------------------------------------------------------------------------------------------------|----------|
| Alkali compounds of preferentially oil soluble sulfonic acids derived from mineral oil (sulfonates 50% oil 50%) | 30       |
| Petrolatum (melting point 116° F.)                                                                              | 30       |
| Carborundum (150-220 mesh)                                                                                      | 30       |
| Emery (80-100 mesh)                                                                                             | 10       |

The grinding compounds according to the present invention are remarkably effective in operation. The compounds have a considerable tendency to remain on the grinding surface. They have a poor lubricating value and are sufficiently viscous to prevent the separation of the abrasive. They may be easily applied to the work and spread over the grinding surface and can be readily removed.

Where a coarse abrasive is used, as in Example II, a good consistency can be obtained without the use of soap. Carborundum is not suitable for use as the coarser abrasive because it scratches the surface and is ineffective for accurate work. The relatively coarse emery is not objectionable on this ac-

count, but on the other hand it is not hard enough to make rapid grinding possible. The combination of the coarse relatively softer abrasive with the fine hard abrasive permits the highly important results of rapid grinding and highly satisfactory finish.

Although the present invention has been described in connection with the details of a specific embodiment thereof, it is not intended that such details shall be regarded as limitations upon the scope of the invention, except in so far as included in the accompanying claims.

I claim:

15. 1. A grinding composition comprising an abrasive, alkali sulfonates derived from oils, and wax.
2. A grinding compound comprising an abrasive, alkali compounds of preferentially oil soluble sulfonates derived from mineral oils, and wax.
3. A grinding compound comprising an abrasive, alkali compounds of preferentially oil soluble sulfonates derived from mineral oils, and petrolatum.
4. A grinding compound comprising an abrasive, alkali sulfonates derived from oils, wax, and oil.
5. A grinding compound comprising an abrasive, alkali compounds of preferentially oil soluble sulfonic acids derived from mineral oil, wax, and oil.
35. 6. A grinding compound comprising an abrasive, alkali compounds of preferentially oil soluble sulfonic acids derived from mineral oil, petrolatum, and oil.
7. A grinding compound comprising an abrasive, alkali sulfonates derived from oils, wax, oil, and fatty acid soap.
40. 8. A grinding compound comprising an abrasive, alkali compounds of preferentially oil soluble sulfonic acids derived from mineral oil, wax, oil, and soap.
45. 9. A grinding compound comprising alkali sulfonates derived from oils, wax, a fine hard abrasive, and a relatively coarser and somewhat softer abrasive.
50. 10. A grinding compound comprising alkali compounds of preferentially oil soluble sulfonic acids derived from mineral oil, wax, a fine hard abrasive, and a relatively coarser and somewhat softer abrasive.
55. 11. A grinding compound comprising alkali sulfonates derived from oils, wax, finely divided carborundum, and somewhat coarser emery.
60. 12. A grinding compound comprising alkali compounds of preferentially oil soluble sulfonic acids derived from mineral oil, wax, finely divided carborundum, and somewhat coarser emery.
65. 13. A grinding compound comprising alkali sulfonates derived from oils, wax, carborundum of about 150 to 220 mesh, and emery of about 80 to 100 mesh.

14. A grinding compound comprising 15% of alkali compounds of preferentially oil soluble sulfonic acids derived from mineral oil, 15% oil, 30% petrolatum, 30% of carborundum of 150 to 220 mesh, and 10% of emery of 80 to 100 mesh.

In testimony whereof I have hereunto set my hand this 5th day of January, 1928.

RICHARD S. McC LAUGHRY.

75

80

85

90

95

100

105

110

115

120

125

130